

## UNITED STATES PATENT OFFICE

1,939,322

## METHOD OF DECORATING SILK FABRICS

Herbert Sieben, Fairlawn, N. J., assignor to Textile Dyeing and Printing Company of America, Inc., Fairlawn, N. J., a corporation of New Jersey

No Drawing. Application April 12, 1932  
Serial No. 665,125

2 Claims. (CL 8—28)

This invention relates to the art of decorating fabrics, and particularly silk fabrics, and it contemplates decorating a silk fabric (by which I mean a fabric including silk, although it may also include other fibers) by first printing thereon in some selected design a resist and then subjecting the fabric to the action of an agent which will so act upon the silk fibers as to effect such a structural change in the areas of the fabric uncovered by the resist that a pronounced decorative contrast between such areas and those covered by the resist will result.

I have found that if the fabric first, as by printing, having the resist deposited thereon in some selected design, is treated with formic acid, preferably concentrated, for a given time and then rid of the resist and the acid the result is that the threads of the areas unprotected by the resist and hence attacked by the acid assume a more straightened form and more compact relation to each other than before the treatment, or than the threads in the resist-protected areas, the straightened form being the result of shrinkage of the threads affected, and when the resist is removed this shrinkage become effective to crinkle the threads in the areas which were protected by the resist. In the preferred practice the gum is previously removed from the silk, as by boiling off the fabric before the treatment, though my invention does not exclude the treatment of goods composed of or including silk yarns boiled off before weaving; when the silk is treated in the raw it is found that the action of the formic acid thereon is retarded, evidently because of the presence of the gum in the silk, wherefore the acid has time not only to act unfavorably on the fibers but to soften the resist.

Further, in the effort to make practical use of this invention in the decorating of fine silk fabrics I have found that formic acid cannot be successfully used on a resist-protected fabric of which the resist substance is the ordinary printing gum, since such resist substance is so readily soluble in acid that satisfactory results are impossible, the resist in places becoming wholly or partially removed by the acid and spoiling the intended design on the fabric because the acid attains access to portions of the fabric assumed to be protected by the resist. Hence my invention further contemplates that specific method which involves depositing the hereinafter specified resist on the fabric and then subjecting the fabric to the formic acid.

In carrying out my invention I prefer to follow this procedure:

If the silk yarns of the fabric are not boiled off previous to weaving the fabric itself is first boiled off, then beamed and tentered. It is then resist-printed, using for the resist a composition consisting of a gum from the acacia class, as gum arabic, and an ordinary printing gum, as shiras or corea, in the approximate proportions of  $\frac{1}{2}$  to  $\frac{1}{3}$ . The printing gum is required in order to afford the composition the necessary plasticity and other qualities which will adapt it to cling to the printing rollers and not be disturbed by the doctor blade of the printing machine when the composition is made to occupy the engraved areas of the printing roller; and the gum arabic or equivalent is present to give the composition the desired resistance to solubility in the presence of the concentrated formic acid.

The fabric is then run through a cold bath of concentrated formic acid so that no portion thereof remains in the bath more than thirty seconds, approximately, it being found that an appreciably less period will not develop the full possible degree of decorative contrast desired and that an appreciably greater period will allow the acid to have some dissolving influence on the resist deposits, with the result that the intended design would be more or less disfigured. The fabric is then run through a cold-water wash, which nullifies the action of the acid on the silk and in fact removes it and dissolves and so also removes the resist both components of which are of course soluble in water; this bath may be still or quiescent so that the formic acid deposited therein may be recovered. Finally it is washed in a running-water bath. The formic acid bath will be improved in its action on the silk if to each liter thereof 1 to 50 cc. of concentrated sulphuric acid is added.

It will be understood that formic acid in concentrated form (or low in water content) is used to reduce the tendency thereof to dissolve the gum of the resist.

One result of my method is that when the fabric is dyed following the treatment the color appears in two different shades, that where the resist was absent presenting a darker shade than that where the resist was present.

Again, if after the formic acid treatment the fabric is weighted and then dyed, the darker areas will be those attacked by the formic acid (or not covered by the resist); this is evidently because the formic acid reduces the responsiveness of the fibers to weighting and since such fibers are consequently deficiently weighted they take up the

dye more readily than the fibers in the areas protected by the resist.

Having thus fully described my invention what I claim is:

6 1. The method of decorating a silk fabric which consists in depositing thereon in a selected design a plastic resist comprising a printing gum and a gum from acacia arabica in substantially the proportions of one-third to two-thirds, respectively, then subjecting the fabric to a formic acid bath, and finally nullifying the action of the acid on the silk and removing the resist.

15

80

85

20

95

25

100

30

105

35

110

40

115

45

120

50

125

55

130

60

135

65

140

70

145

75

150

2. The method of decorating a silk fabric which consists in depositing thereon in a selected design a plastic resist comprising a printing gum and a gum from acacia arabica in substantially the proportions of one-third to two-thirds, respectively, then subjecting the fabric to a concentrated formic acid bath so that each part of the fabric will be so subjected for about thirty seconds, and finally nullifying the action of the acid on the silk and removing the resist.

HERBERT SIEBEN.